

Patented June 25, 1929.

1,718,642

# UNITED STATES PATENT OFFICE.

JOHN A. GANN, OF MIDLAND, MICHIGAN, ASSIGNOR TO THE DOW CHEMICAL COMPANY, OF MIDLAND, MICHIGAN, A CORPORATION OF MICHIGAN.

## LIGHT-METAL ALLOY.

No Drawing. Application filed October 18, 1922, Serial No. 595,277. Renewed September 1, 1926.

The present improved alloy is one in which magnesium is the predominant element, such metal being preferably present in excess of 80 per cent, as prescribed in U. S. Patent No. 5 965,485 to Pistor et al., dated July 26, 1910. The other added metals include copper, aluminum and cadmium, the copper being added in amounts greater than those of aluminum and cadmium. 10 As noted in Reinglass treatise on "Alloys" (see page 175), the French patent to Walter Rübel, No. 407,814, dated October 12, 1909, such patent corresponding in part to his U. S. Patent No. 982,022, dated January 17, 1911, 15 suggests that the zinc in this patentee's magnesium-zinc formula may be partly replaced by copper or entirely by aluminum and copper. One illustrative formula of the latter ternary alloy is as follows, viz, magnesium 90 per cent, copper 9 per cent and aluminum 1 per cent. 20 I have found that magnesium-copper alloys are not very strong and furthermore are not particularly good for casting purposes 25 and that the addition of a little aluminum, in accordance with the Rübel formula just cited, greatly improves both the strength and the casting properties of such magnesium-copper alloy. On the other hand, the addition of a 30 little cadmium to such magnesium-copper alloy does not appreciably improve the alloy; in fact, it often gives a very inferior casting. 35 If, however, instead of dealing with such magnesium-copper alloy, we take a magnesium-copper-aluminum alloy of approximately the composition described by Rübel and add a small amount of cadmium, I have found that 40 an alloy is produced that is considerably better than the original ternary alloy. In other words, the resulting quarternary magnesium-copper-aluminum-cadmium alloy presents superior qualities both from the standpoint of strength and toughness and that of casting and general workability. 45 The composition of my improved alloy will now be fully described and particularly pointed out in the claims, it being understood that the following description sets forth but several of the various ways in which 50 the principle of the invention may be carried out. The ranges of composition that have been found satisfactory for use in my improved quarternary alloy are as follows, viz, copper 1 to 12 per cent (4 to 8 per cent being preferred), aluminum 1 to 4 per cent (1 to 2 per cent being preferred), cadmium 1 to 4 per cent (2 to 3 per cent being preferred), and magnesium constituting the balance. 55 A specific formula that has proven very 60 satisfactory, both in test and actual use, is as follows, viz, magnesium 92 per cent, copper 4 per cent, aluminum 2 per cent, cadmium 2 per cent. The physical properties of this particular alloy have been determined 65 to be as follows, viz, tensile strength 20,000 to 22,000 lbs. per square inch; thermal conductivity 0.30; single-blow impact-toughness 70 55; and Brinell hardness 45. As compared with other commercial light metal alloys 75 wherein magnesium is the predominant ingredient, my new alloy would appear to have approximately the same tensile strength combined with a somewhat greater toughness, as indicated by the single-blow impact number, 75 a somewhat lower Brinell hardness, and a much higher thermal conductivity. 80 Accordingly, it would appear that the addition of cadmium to a ternary magnesium-copper-aluminum alloy of the type in hand, 85 wherein the amount of copper is in excess of that of aluminum, materially increases the strength and toughness of the resulting product and so presents an effect that would be wholly unsuspected from the effect of adding cadmium to a binar magnesium-copper alloy. It will be understood that the physical properties of my improved alloy may be modified by the additions of small amounts of other metals such as zinc and tin. Where 90 zinc is thus employed, the amount thereof will desirably be kept within the range where such zinc will dissolve in the magnesium, i. e., enter into solid solution. With this in mind, the amount of zinc recommended is from 95 0.30 per cent to 0.65 per cent, only, while the amount of tin, where this metal is added, should not greatly exceed 1 per cent of the total. 100 Other modes of applying the principle of my invention may be employed instead of the one explained, change being made as regards the materials employed, provided the ingredients stated by any of the following claims or the equivalent of such stated ingredients be employed. 105 I therefore particularly point out and distinctly claim as my invention:— 1. As a new product, an alloy consisting of magnesium, copper, aluminum and cad- 110

mium, wherein the magnesium largely predominates and the amount of the copper ranges from approximately 3 to 12 per cent, the amount of copper exceeding that of 5 aluminum and the latter as well as the cadmium being present in substantial amounts.

2. As a new product, an alloy consisting of magnesium, copper, aluminum and cadmium, wherein the magnesium is in excess of 10 80 per cent and the amount of the copper ranges from approximately 3 to 12 per cent, the amount of copper being approximately twice that of aluminum and the latter as well as the cadmium being present in substantial 15 amounts.

3. As a new product, an alloy consisting of magnesium, copper, aluminum and cad-

mium, wherein the magnesium largely predominates, and the copper exceeds the aluminum, the copper being from 3 to 12 per cent, 20 the aluminum from 1 to 4 per cent, and the cadmium from 1 to 4 per cent of the total.

4. As a new product, an alloy containing magnesium, copper, aluminum and cadmium, wherein the magnesium largely predominates, 25 the copper being from 4 to 8 per cent, the aluminum from 1 to 2 per cent, and the cadmium from 2 to 3 per cent of the total.

5. As a new product, an alloy containing approximately 92 per cent of magnesium, 30 4 per cent of copper, 2 per cent of aluminum and 2 per cent of cadmium.

Signed by me, this 14 day of October, 1922.  
JOHN A. GANN.